

## UNITED STATES PATENT OFFICE.

JOHN G. CAPSTAFF, OF ROCHESTER, NEW YORK, ASSIGNEE TO EASTMAN KODAK COMPANY, OF ROCHESTER, NEW YORK, A CORPORATION OF NEW YORK.

## REVERSAL PROCESS.

No Drawing.

Application filed January 31, 1925. Serial No. 6,148.

This invention relates to an improved photographic reversal process and more particularly to a step therein for preventing reversal. The improved step will be described as incorporated in the process covered by my Patent No. 1,480,708, granted July 3, 1923. The principal steps of that process were successively, exposure, development, removal or bleaching of the silver image, clearing, controlled re-exposure, re-development and a final fixing. If a tendency to re-reversal was found by test to take place at the second development, there was introduced a step to overcome this tendency, this step comprising an alkali bath prior to re-exposure and re-development.

I have since discovered cases of re-reversal that were not satisfactorily overcome by this treatment and I have further discovered that these occurred when a fresh bleaching or reversing bath, such as is described in step 4 of the patent, was used for the first time; but that the tendency disappeared after the bath had been used a short time. Further research disclosed the fact that this tendency is not found when there is present in the bleaching or reversing bath a small amount of a soluble silver salt.

My improved step consists in the conditioning of this reversal or bleaching bath by the purposeful addition thereto of such a solution. This conditioning may be accomplished in various ways, of which the following is an instance. To one liter of a bath made in accordance with the formula given in step 4 of said patent may be added 2½ cc. of a 10% solution of silver nitrate. A second method of introducing the soluble silver salt, useful when a continuous machine such as is described in my application Serial No. 616,846, filed February 3, 1923, is used is to run a strip of waste film through the machine including the bleaching bath prior to its use in regular work. This would be done by fogging such a strip and using it as a leader for the regular film, then drawing it through the developing and bleaching baths. The action of the bleaching bath on the developed silver of the waste strip would introduce silver salt into the bath. The length of such a strip would have to be ascertained by experiment under the conditions present in the actual apparatus. A third

way of attaining the desired object is to add to a newly prepared bath a quantity of liquid from a used or exhausted bleaching bath and this quantity would also, of course, have to be determined by experiment and the actual condition and content of the used bath. However, the first method mentioned gives a precise step available to those without experience.

The re-reversal mentioned is usually a combination of negative and positive images and not a complete re-reversal. It tends to appear most strongly when there was originally an under-exposure in the camera, since in such cases there is little silver in the developed image and the bleaching bath is slow to acquire a silver salt from its action on this thin image. If the original developed image is very dense, the tendency to re-reverse disappears much more quickly because of the rapid formation of the silver salt in the bleaching bath.

This invention is of particular use in the reversal process described in my patent in which the re-exposure is controlled and in which all the sensitive silver salts are not usually redeveloped; because re-reversal cannot occur in the usual reversal processes wherein all the sensitive silver salts are redeveloped.

The theory underlying the cause and prevention of this type of re-reversal is obscure.

As stated in the patent, the preferred reversing bath is as follows:

|                                      | Parts. |
|--------------------------------------|--------|
| Potassium permanganate (4% solution) | 1 00   |
| Sulfuric acid (20%)                  | 1      |
| Water                                | 20     |

As described in the patent, the bath contains about 1% of sulphuric acid, and the silver salt formed in the bleaching operation is silver sulfate. When silver nitrate is added to the bath it is transformed into silver sulfate. When silver salts less soluble than the sulfate, such as the halides, are added, the result is not obtained. It appears to be necessary to use a salt which will be transformed into the salt of the acid of the bleaching bath, in this case, the sulfate.

The bath as used substantially contains silver salt to produce a saturated solution of

silver sulfate in the bath. The solubility of the sulfate increases with the acidity of the bath and as the acidity of the bath may vary, as was stated in the patent, the amount of sulfate may correspondingly vary.

In each of the various methods mentioned above it will be seen that this salt is incorporated in the bath when it is initially used for its intended purpose.

10 Having thus described my invention what I claim is new and desire to secure by Letters Patent is:

1. The method of conditioning an acid bath for use in a photographic reversal process for bleaching a silver image preparatory to re-development that comprises the incorporation therein of a silver salt corresponding to the acid of the bath.

2. The method of conditioning a bath containing sulfuric acid for use in a photographic reversal process for bleaching a silver image preparatory to re-development that comprises the incorporation therein of silver sulfate.

25 3. The method of conditioning a bath comprising a permanganate and sulfuric acid for use as a bleaching bath for a silver image preparatory to re-development thereof

that comprises the incorporation therein of silver sulfate.

4. In a photographic reversal process comprising successively submitting a carrier with a silver image to an acid bleaching bath and to a redeveloping bath, the improved step that comprises using for bleaching a bath that has initially present a silver salt of the acid of the bath.

5. In a photographic reversal process comprising successively submitting a carrier with a silver image to a bleaching bath containing sulfuric acid and then to a redeveloping bath, the improved step that comprises using for bleaching a bath that has silver sulfate initially present.

6. In a photographic reversal process comprising successively submitting a carrier with a silver image to a bleaching bath containing a permanganate and sulfuric acid and then to a redeveloping bath, the improved step that comprises using for bleaching a bath that has silver sulfate initially present.

Signed at Rochester, New York, this 29th day of January 1925.

JOHN G. CAPSTAFF.

silver sulfate in the bath. The solubility of the sulfate increases with the acidity of the bath and as the acidity of the bath may vary, as was stated in the patent, the amount of sulfate may correspondingly vary.

In each of the various methods mentioned above it will be seen that this salt is incorporated in the bath when it is initially used for its intended purpose.

10 Having thus described my invention what I claim is new and desire to secure by Letters Patent is:

1. The method of conditioning an acid bath for use in a photographic reversal process for bleaching a silver image preparatory to re-development that comprises the incorporation therein of a silver salt corresponding to the acid of the bath.

2. The method of conditioning a bath containing sulfuric acid for use in a photographic reversal process for bleaching a silver image preparatory to re-development that comprises the incorporation therein of silver sulfate.

25 3. The method of conditioning a bath comprising a permanganate and sulfuric acid for use as a bleaching bath for a silver image preparatory to re-development thereof

that comprises the incorporation therein of silver sulfate.

30 4. In a photographic reversal process comprising successively submitting a carrier with a silver image to an acid bleaching bath and to a redeveloping bath, the improved step that comprises using for bleaching a bath that has initially present a silver salt of the acid of the bath.

35 5. In a photographic reversal process comprising successively submitting a carrier with a silver image to a bleaching bath containing sulfuric acid and then to a redeveloping bath, the improved step that comprises using for bleaching a bath that has silver sulfate initially present.

40 6. In a photographic reversal process comprising successively submitting a carrier with a silver image to a bleaching bath containing a permanganate and sulfuric acid and then to a redeveloping bath, the improved step that comprises using for bleaching a bath that has silver sulfate initially present.

45 Signed at Rochester, New York, this 29th day of January 1925.

JOHN G. CAPSTAFF.

#### Certificate of Correction.

It is hereby certified that in Letters Patent No. 1,600,797, granted September 21, 1926, upon the application of John G. Capstaff, of Rochester, New York, for an improvement in "Reversal Processes," an error appears in the printed specification requiring correction as follows: Page 1, lines 3 and 4, for the word "reversal" read *re-reversal*; and that the said Letters Patent should be read with this correction therein that the same may conform to the record of the case in the Patent Office.

Signed and sealed this 19th day of October, A. D. 1926.

[SEAL.]

WM. A. KINNAN,  
*Acting Commissioner of Patents.*

**Certificate of Correction.**

It is hereby certified that in Letters Patent No. 1,600,797, granted September 21, 1926, upon the application of John G. Capstaff, of Rochester, New York, for an improvement in "Reversal Processes," an error appears in the printed specification requiring correction as follows: Page 1, lines 3 and 4, for the word "reversal" read *re-reversal*; and that the said Letters Patent should be read with this correction therein that the same may conform to the record of the case in the Patent Office.

Signed and sealed this 19th day of October, A. D. 1926.

[SEAL.]

WM. A. KINNAN,  
*Acting Commissioner of Patents.*